

## UNITED STATES PATENT OFFICE

2,306,033

## BEARING

Adolf Beck and Walter Buchmann, Bitterfeld, Germany, assignors, by mesne assignments, to Magnesium Development Corporation, a corporation of Delaware

No Drawing. Application August 22, 1939, Serial No. 291,322. In Germany August 22, 1938

4 Claims. (Cl. 308—242)

This invention relates to bearings. Certain commercial magnesium base alloys containing aluminium and zinc have occasionally been used in the production of bearings, which however have given good results only when subjected to small loads, that is to say, in a limited field of application. Thus for example, the attempt to mount camshafts in crank-cases made of these alloys has been successful. This is due to the fact that even pure magnesium itself has relatively good sliding properties, probably due to its hexagonal crystal structure. The known commercial magnesium alloys, however, are unsuitable for bearings which are exposed to heavier pressures and, in particular, higher sliding speeds. They lack, in particular, the essential property of being able to form, through running-in, a bearing surface which is uniformly loaded; in the event of the shaft being tilted, and particularly if lubrication should fail temporarily, local increases in temperature therefore readily occur on the bearing surfaces, which lead to the rapid destruction of the bearing. The so-called emergency running properties of bearings made from such magnesium base alloys are therefore unsatisfactory.

It has now been ascertained, in accordance with the present invention, that the properties necessary to the more extensive use of magnesium base alloys as bearing metal, are obtained by the use of alloys of magnesium with the metals lead and/or cadmium, both of which form solid solutions with magnesium up to relatively high contents, and the presence of which not only does not reduce, but rather increases, the plastic properties of the magnesium.

Broadly, the present invention provides a bearing metal alloy, consisting of magnesium and containing up to 28% of lead or up to 35% of cadmium, or up to 35% of lead and cadmium jointly. When the foregoing percentages are exceeded, the bearing properties of the resultant alloys deteriorate.

The bearing metal alloys of the present invention preferably contain 15 to 20% of lead and/or 7 to 12% of cadmium. Silver, bismuth and tin also may advantageously be present in the foregoing alloys in amounts of up to 12%, but only provided that the total content of alloy formers in the alloys does not exceed about 35%.

By comparison with hitherto proposed light bearing metal alloys, the bearing metal alloys of the present invention possess more favourable running-in properties, due to their enhanced

plastic properties. They are quite generally suitable for bearing purposes for light to medium loads and, in this range of use, are equivalent in respect to their sliding properties to known heavy metal bearing alloys, over which latter they have the important advantage of lower specific gravity.

For heavier loads, such as those occurring in internal combustion engines, the alloys of the present invention are somewhat deficient in respect of fatigue strength and heat strength. However, these properties can be substantially improved without unduly impairing the plastic properties and the ability to form good running surfaces, by additionally incorporating with the alloys, cerium in amounts of from about 0.5 to 10%. The amount of the cerium addition depends not only on the intended use, but also on the amount of other alloy formers contained in the alloy. The increase in strength at elevated temperatures becomes appreciable, for example in the case of alloys having a high lead content, only when the added amount of cerium is high.

The following are examples of bearing metal alloys in accordance with the invention:

I. 18% of lead, remainder magnesium.

II. 12% of lead, 8% of cadmium, remainder magnesium.

III. 7% of lead, 7% of cerium, remainder magnesium.

IV. 10% of cadmium, 5% of cerium, remainder magnesium.

We claim:

1. A bearing made from a magnesium base alloy containing between about 15 and about 20% of lead, the balance being substantially magnesium.

2. A bearing from a magnesium base alloy containing between about 1 and about 28% of lead, further up to about 12% of at least one metal of the group consisting of silver, bismuth and tin, and between about 0.5 and about 10% of cerium, the total content of the alloying constituents stated not exceeding about 35%, and the balance being substantially magnesium.

3. A bearing made from a magnesium base alloy containing about 18% of lead, the balance being substantially magnesium.

4. A bearing made from a magnesium base alloy, said alloy containing between about 1 and about 28 per cent lead, the balance being substantially magnesium.

ADOLF BECK.  
WALTER BUCHMANN.